

## UNITED STATES PATENT OFFICE

2,639,990

PROCESS FOR IMPROVING THE WHITENESS  
OR COLOR OF MATERIALS AND PRODUCTS  
RESULTING THEREFROMJohn David Kendall and George Frank Duffin,  
Ilford, England, assignors to Ilford Limited,  
Ilford, England, a British companyNo Drawing. Application May 29, 1950, Serial  
No. 165,116. In Great Britain June 3, 1949

13 Claims. (Cl. 95—7)

**1** This invention relates to a process for the improvement of natural or synthetic fibrous materials and of films of natural or synthetic colloid materials. Within these terms are to be understood textile materials generally, in the form of filaments, threads, yarns, woven or knitted fabrics, made of cotton, silk, wool, hemp or flax, or of synthetic materials such as regenerated cellulose, cellulose nitrate, cellulose acetate, cellulose propionate, cellulose butyrate and mixed cellulose esters as, for instance, cellulose acetate-butyrate and cellulose acetate-propionate, nylon and similar synthetic linear polyamides, vinyl derivatives such as vinyl esters, acetals, chlorides and other polymeric colloid materials including mixed polymers and interpolymers of vinyl derivatives. Also included are natural fibrous materials such as wood pulp and synthetic fibrous materials made of any of the foregoing types of synthetic compound not in textile form. The terms also include sheet materials formed from any of the foregoing synthetic materials, e. g. films of cellulose acetate, cellulose nitrate, cellulose acetate-butyrate and the like, or formed from compacted fibres, e. g. paper, cardboard, felt and the like, or from natural colloids such as gelatin.

The foregoing materials and materials of similar character are hereinafter referred to for brevity as "fibres and films."

According to the present invention a process for improving fibres and films comprises applying thereto a small quantity of a fluorescent compound of the general formula:



wherein  $R_1$  is a hydrogen atom, hydrocarbon group or substituted hydrocarbon group,  $Ar_1$  is an aromatic residue, e. g. phenyl or naphthyl, which may contain any of the substituents hydroxy, alkoxy, hydroxyalkyl, amino, hydrocarbon-substituted-amino or acylamino groups or halogen atoms and  $Ar_2$  is an aromatic nucleus which may contain any substituent groups, e. g. substituent hydrocarbon, hydroxy, alkoxy, hydroxyalkyl, amino, hydrocarbon-substituted-amino, acylamino, sulphonic, carboxylic, or cyano groups, which compound is colourless in aqueous or ethyl alcoholic solution. By the term "colourless in aqueous or ethyl alcoholic solution" is meant that a solution of the compound in water or ethyl alcohol has an absorption maximum not greater than 4000 Å. The preferred compounds

are those in which the absorption maximum does not exceed 3900 Å.

The foregoing definition of the compounds does not include compounds in which  $R_1$  or  $Ar_2$  contains a nitro substituent, or in which  $Ar_1$  contains a sulphonic carboxylic nitro or cyano group since those compounds do not fluoresce.

Compounds of the foregoing formula in which  $R_1$  or the group  $Ar_2$  are hydrocarbon radicles containing substituent carboxylic or sulphonic acid groups are for many purposes particularly favourable, since they form alkali metal and ammonium salts which are substantive to practically the whole range of fibres and films referred to above. The free carboxylic and sulphonic acids are substantive to protein and polyamide fibres and films, but for the other materials, e. g. cellulosic materials such as cotton and paper, and cellulose acetate materials, the alkali salts are generally preferred.

Examples of water-insoluble compounds which may be used in accordance with the present invention are:

|                                                       | M. P., °C. |
|-------------------------------------------------------|------------|
| 1 : 3-diphenyl pyrazoline                             | 152        |
| 1 : 3 : 5-triphenyl pyrazoline                        | 145        |
| 1-phenyl-3-m-tolyl pyrazoline                         | 77         |
| 1-m-tolyl-3-phenyl pyrazoline                         | 88         |
| 1-phenyl-3-p-bromophenyl pyrazoline                   | 130        |
| 1 : 3-di-m-tolyl pyrazoline                           | 120        |
| 1 : 3-diphenyl-5-methyl pyrazoline                    | 105        |
| 1 : 5-diphenyl-3-p-tolyl pyrazoline                   | 154        |
| 1 : 5-diphenyl-3-p-methoxyphenyl pyrazoline           | 142        |
| 1 : 5-diphenyl-3-p-ethoxyphenyl pyrazoline            | 131        |
| 1 : 5-diphenyl-3-p-phenoxyphenyl pyrazoline           | 162        |
| 1 : 5-diphenyl-3-(p-phenyl)phenyl pyrazoline          | 205        |
| 1 : 5-diphenyl-3-(p-ethoxy-m-methyl)phenyl pyrazoline | 135        |
| 1-phenyl-3 : 5-di(p-chlorophenyl)phenyl pyrazoline    | 151        |
| 1 : 3-diphenyl-5-p-methoxyphenyl pyrazoline           | 124        |
| 35 1-phenyl-3-p-methoxyphenyl-5-p-tolyl pyrazoline    | 127        |
| 1-phenyl-3-p-tolyl-5-p-methoxyphenyl pyrazoline       | 141        |
| 1-phenyl-3 : 5-di(p-methoxy)phenyl pyrazoline         | 147        |
| 1 : 4-di(1' : 3'-diphenyl pyrazolinyl-5)benzene       | 290        |

Examples of water-soluble compounds which can be used are:

|                                                              |  |
|--------------------------------------------------------------|--|
| 40 1-(p-sulphophenyl)-3-phenyl pyrazoline                    |  |
| 1-(p-sulphophenyl)-3 : 5-diphenyl pyrazoline                 |  |
| 1-p-phenoxy-m-sulphophenyl-3-phenyl pyrazoline               |  |
| 1-p-sulphophenyl-3-phenyl-5-methyl pyrazoline                |  |
| 1-p-sulphophenyl-3-p-tolyl-5-phenyl pyrazoline               |  |
| 1-p-sulphophenyl-3-p-methoxyphenyl-5-phenyl pyrazoline       |  |
| 1-p-sulphophenyl-3-p-ethoxyphenyl-5-phenyl pyrazoline        |  |
| 1-p-sulphophenyl-3-p-phenoxyphenyl-5-phenyl pyrazoline       |  |
| 1-p-sulphophenyl-3-(p-phenyl)phenyl-5-phenyl pyrazoline      |  |
| 1-p-sulphophenyl-3-phenyl-5-p-methoxyphenyl pyrazoline       |  |
| 1-p-sulphophenyl-3-p-tolyl-5-p-methoxyphenyl pyrazoline      |  |
| 1-p-sulphophenyl-3 : 5-di(methoxyphenyl) pyrazoline          |  |
| 1 : 4-di(1'-p-sulphophenyl-3'-phenyl-pyrazolinyl-5)benzene   |  |
| 1-m-sulphophenyl-3 : 5-di(p-chlorophenyl) pyrazoline         |  |
| 50 1-m-sulphophenyl-3-(p-phenyl)phenyl-5-phenyl pyrazoline   |  |
| 1-m-sulphophenyl-3 : 5-diphenyl pyrazoline                   |  |
| 1-(p-methyl-m-sulpho)phenyl-3 : 5-diphenyl pyrazoline        |  |
| 1-(p-methyl-o-sulpho)phenyl-3 : 5-diphenyl pyrazoline        |  |
| 1-(4'-sulpho-2' : 5'dichlorophenyl-3 : 5-diphenyl pyrazoline |  |
| 1-(4 : 8-disulphonaphthalyl-2)-3 : 5-diphenyl pyrazoline     |  |
| 55 1-p-sulphophenyl-3-phenyl-5- $\alpha$ -furyl pyrazoline   |  |
| 1 : 3-diphenyl-5-o-sulphophenyl pyrazoline                   |  |
| 1-p-tolyl-3-phenyl-5-o-sulphophenyl pyrazoline               |  |
| 1-p-acetamidophenyl-3-phenyl-5-o-sulphophenyl pyrazoline     |  |

The preferred compounds according to the

present invention are those in which the pyrazoline contains a sulphonphenyl group in the 1-position and contains in the 3- and 5-positions phenyl groups or substituted phenyl groups.

The compounds may be prepared by various methods. One method is described in co-pending application Serial No. 165,118, filed on even date herewith. A second method consists in the condensation of a Mannich reaction product (obtained from an acetophenone with formaldehyde and an amine) with an aryl hydrazine, and a third method is the condensation of a ketone of the type  $\text{Ar}-\text{CO}-\text{C}(\text{R})=\text{CH}_2$  with an aryl hydrazine.

Compounds of the foregoing general formula which are colourless, white or pale yellow have been found to possess a strong bluish fluorescence in daylight and a slightly less fluorescence in incandescent electric or similar light, and on application to fibres and films they impart such fluorescence to them. The effect of applying these compounds to fibres and films is to impart a degree of brilliance to them which is attractive and useful. Applied to materials which are allegedly white, but of which the whiteness has a slight tinge of yellow or brown, the compounds serve to "kill" the yellow or brown tinge so that the apparent whiteness of the materials is very appreciably enhanced. This application of the materials is of especial importance, and the present invention is therefore particularly concerned with the application of the compounds to such "off-white" fibres and films. It is a special advantage of the compounds of this invention, and especially those in which  $\text{R}_1$  or  $\text{Ar}_2$  contain a sulphon group, that they impart a very desirable whiteness to wool fibres, the effect being a strong resistance to fading under the action of light and a strong resistance to laundering.

Applied to dyed textile materials the compounds have the effect of improving the apparent purity of the colour.

Very small quantities of the compounds are sufficient to achieve the desired improvement in the materials. Thus the whiteness of textile materials, paper and the like can be very considerably enhanced by treating the materials with a solution of one of the said compounds, in water or an organic solvent, e. g. at a solution concentration of 1 part in 5000 to 1 part in 100,000. Applied to wool, the compound in which  $\text{R}_1$  or  $\text{Ar}_2$  contains a sulphon acid group may be used from weakly acid solution or even neutral solution and are substantive to wool from such solutions.

In order to convert the solution concentration of 1 in 5,000 and 1 in 100,000 to percent of compound absorbed by weight it must be assumed that the ratio of fibre to dye bath ranges from 1 to 10 to 1 to 50 and that the dye bath is operated to exhaustion. Both of these assumptions are customary dyeing practice. Thus, taking the strongest solution envisaged, 1 in 5,000 and the greatest ratio of dye bath to fibre (50:1), one obtains the conditions in which the greatest amount of dye will be absorbed. In this case 50 parts of dye bath will contain 0.01 part of fluorescent compound, i. e., one part of fibre takes up 0.01 part of fluorescer, which is 1%.

Taking, on the other hand, the most dilute bath of 1 in 100,000 and the lowest ratio of fibre (10:1), the 10 parts of bath will contain 0.0001 part of fluorescer, i. e., one part of fibre takes up 0.0001 part of fluorescer, which is 0.01%. Therefore from the figures of 1 to 5,000 and 1 to 100,000

and the normal dyeing practice an absorption computation of 0.01 to 1% is calculated.

In the case of fibres or films which are not in their natural state, the compounds of this invention may be applied thereto at any stage in the manufacture of such materials. Thus in the production of artificial filaments, fibres or films by the extrusion or casting of colloid compositions, the compounds of this invention may be incorporated in such compositions before extrusion or casting so that they are uniformly dispersed throughout the products.

Alternatively the preferred fibres or films may be treated with solutions of the compounds. Thus in the treatment of textile materials the compounds may be included in any of the liquids commonly employed for dyeing, scouring, dressing and the like, and this invention includes compositions for application to textiles for such purposes which include a compound of the foregoing formula in conjunction with a textile dye, detergent or other material used for treating textiles. The compounds may be applied to the materials after the normal processes of their manufacture have been completed, for example by including the compounds in domestic washing preparations.

In the case of paper and similar materials the compounds may be applied to the wood pulp or rag-fibre before such material is made into paper, or during the paper-making operation, or may be applied as a solution directly to the raw paper, or may be applied in a dressing composition, e. g. a baryta coating, applied to the paper.

The compounds referred to above in which neither  $\text{R}_3$  nor  $\text{Ar}_2$  contains a sulphon or carboxylic group fluoresce strongly in organic solvents and may be applied to protein and polyamide fibres from an organic solvent or aqueous organic solvent, e. g. aqueous ethyl alcohol or aqueous acetic acid. These compounds, by reason of their solubility in organic solvents, are also especially adapted for inclusion in solutions of cellulose acetate and similar materials which are to be extruded or cast to form fibres or films.

One important application of the invention is in the treatment of photographic prints where application of a solution of a compound of the foregoing general formula has the effect of whitening the highlights of the print. Considerable effort has hitherto been directed to the production of prints having brilliant highlights, and the present invention provides a simple method whereby this result may be achieved. However, the compounds may, if desired, be incorporated in the photographic emulsions, or sub-coat or super-coat layers, prior to coating such layers to form the photographic element.

In the case of prints made on paper carrying silver bromide emulsions, the prints normally have a "warm" tone, but by treatment with a compound according to this invention the tone may be changed to resemble very closely the cold tone commonly associated with prints made on paper coated with silver chloride emulsions.

The compounds of this invention may also be applied to films coated on supports, for example to finished photographic films or plates where the gelatin film takes up the compound and is thereby caused to fluoresce and the photographic image to appear colder in tone.

What we claim is:

1. A process for improving fibres and films which comprises applying thereto a dispersion

5

in a liquid medium of a white fluorescent compound of the general formula:



wherein R<sub>1</sub> is selected from the class consisting of the hydrogen atom, alkyl, unsubstituted phenyl and phenyl containing alkyl, alkoxy, chloro and sulphonate substituents, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents, so that the said fibres and films absorb 0.01 to 1% by weight of the said compound.

2. A process for improving fibres and films which comprises applying thereto an aqueous solution of a white fluorescent compound of the general formula:



wherein R<sub>1</sub> is selected from the class consisting of the hydrogen atom, alkyl, unsubstituted phenyl and phenyl containing alkyl, alkoxy, chloro and sulphonate substituents, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents, so that the said fibres and films absorb 0.01 to 1% by weight of the said compound.

3. A process for improving fibres and films which comprises applying thereto an aqueous solution of a fluorescent compound of the general formula:



wherein R<sub>1</sub> is a sulphonated phenyl group, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents, so that the said fibres and films absorb 0.01 to 1% by weight of the said compound.

4. A process for improving the whiteness of wool fibres and woollen textile materials which comprises applying thereto an aqueous solution of a compound of the general formula:



wherein R<sub>1</sub> is selected from the class consisting of the hydrogen atom, alkyl, unsubstituted

10

phenyl and phenyl containing alkyl, alkoxy, chloro and sulphonate substituents, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents, so that the said fibres and films absorb 0.01 to 1% by weight of the said compound.

5. A process for improving the whiteness of wool fibres and woollen textile materials which comprises applying thereto an aqueous solution of a compound of the general formula:



wherein R<sub>1</sub> is a sulphonated phenyl group, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents, so that the said fibres and films absorb 0.01 to 1% by weight of the said compound.

6. Thin flexible organic materials for use in textiles and photographic printing containing 0.01 to 1% of a white fluorescent compound of the general formula:



wherein R<sub>1</sub> is selected from the class consisting of the hydrogen atom, alkyl, unsubstituted phenyl and phenyl containing alkyl, alkoxy, chloro and sulphonate substituents, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents.

7. Woollen textile materials having adsorbed thereto 0.01 to 1% of a white fluorescent compound of the general formula:



wherein R<sub>1</sub> is selected from the class consisting of the hydrogen atom, alkyl, unsubstituted phenyl and phenyl containing alkyl, alkoxy, chloro and sulphonate substituents, Ar<sub>1</sub> is selected from the class consisting of unsubstituted phenyl and phenyl containing halogen, alkyl, alkoxy and phenoxy substituents, and Ar<sub>2</sub> is selected from the class consisting of unsubstituted phenyl and phenyl containing halogen, alkyl, sulphonate and acetylaminio substituents.

8. Woollen textile materials having adsorbed

75

